

Oct. 8, 1935.

C. J. KATZE-MILLER

2,016,447

PROCESS OF MAKING CONDUITS

Filed Jan. 14, 1933



MATTED MASS OF  
LEATHER AND WOOD FIBERS  
IMPREGNATED WITH  
WATERPROOFING MATERIAL

INVENTOR  
CARLTON J. KATZE-MILLER  
BY

*Arthur R. Woerck*  
ATTORNEY

## UNITED STATES PATENT OFFICE

2,016,447

## PROCESS OF MAKING CONDUITS

Carlton J. Katze-Miller, Milwaukee, Wis., assignor  
to Line Material Company, South Milwaukee,  
Wis., a corporation of Delaware

Application January 14, 1933, Serial No. 651,709

4 Claims. (Cl. 92—21)

This invention relates to waterproof fibrous material and to the process of making the same, and is particularly directed to the manufacture of conduits, pipes, fiber board, wall board and various insulating materials.

In the manufacture of articles such as electrical conduits from fibrous materials as wood pulp, such, for instance, as that obtained from paper stock, it is the customary practice to dis-  
10 integrate the stock by the use of a beater and conduct the web from a web forming machine to a rotary mandrel where it is wound into a tube of the desired thickness, the mandrel being subsequently withdrawn and the tube dried. The  
15 stock is of such a character and contains such an amount of water that the fibers felt or mat to produce a substantially homogeneous fibrous tube. The tubes thus formed are dried and subsequently impregnated with a waterproofing agent.

These conduits formed from wood pulp have a certain amount of strength and a certain life even when used in underground work, such as housing electric wires, cables, etc., but they are  
25 expensive as the cost of the wood pulp, whether from paper stock or not, is a fairly large item. There is a decided need for a conduit which is materially cheaper, which has a long life, and which is very strong.

30 This invention is designed to provide a fibrous product, such as a conduit, for instance, and a method of making the same, which obviates the disadvantages hereinbefore enumerated and which provides a fibrous conduit which is very  
35 much stronger than one formed of wood pulp, which has a longer life, and which is considerably cheaper than the heretofore known type of wood pulp conduits.

40 It has been found that leather fiber can be used to greatly cheapen the process as the waste leather scrap from the leather industry, the tanneries, shavings and scraps from shoe factories, or other factories for producing leather or leather articles, is usually discarded, frequently the factories paying to have it hauled away. This leather scrap can, therefore, be obtained for almost nothing and in great abundance.

45 This invention contemplates the use of leather fiber, either alone, or mixed with wood fiber in the production of conduits and other fibrous products.

In practicing this invention it is advisable to first thoroughly wash the leather scrap with water, preferably slightly warmed, to remove the

salts that the leather carries from the tanning. Thereafter the washed leather scrap is put into a beater, such as used in paper manufacturing, and, if wood pulp is used, paper stock or other source of wood pulp is added to the beater.

In one mode of carrying out the invention, the stock of leather and wood pulp is beaten with water. The beating continues until the fibrous mass conforms to the standard sheet test. The fibrous mass then goes through the conventional 10 forming machines, such as conduit forming machines, in the usual manner.

Thereafter the conduit or other article is thoroughly dried, preferably the drying starting at a moderate temperature and the temperature 15 being gradually increased.

After drying the conduit or other article it is impregnated with a waterproofing agent. Various impregnating compounds may be used, and, without limiting the invention thereto, a few 20 may be mentioned, viz:—asphalt, pitch, wax, lignin (which is found in the waste sulphite liquors from paper making), casein, rosin, or paraffin. The material when impregnated with casein may have the casein subsequently hardened by the use of formaldehyde or other hardening material. The impregnating preferably is conducted under pressure.

With certain impregnating material, such as asphalt, pitch, etc., it is preferable to immediately 30 spray the conduit or article after impregnating to cause it to become chilled suddenly to prevent distortion while it is hot.

In another mode of carrying out this invention leather fiber alone may be employed. Impregnation is vastly more difficult, however, where leather fiber alone is used. It has been found that the addition of even a small amount of wood fiber greatly facilitates impregnation.

This invention, therefore, contemplates the use 40 of leather fiber in the formation of conduits or other articles, with or without the use of wood fiber, and if wood fiber is used, with the percentage of wood fiber running all the way from 45 a small percent with reference to the leather fiber to a large percent.

The accompanying drawing shows a finished conduit.

I have found that a leather fiber product 50 shrinks very much on drying, whereas a wood fiber product has relatively little shrinkage during the drying. Further, a wood fiber product is easily impregnated with a waterproofing agent, whereas a wholly leather fiber product is diffi-

cultly impregnated with a waterproofing agent.

From numerous experiments I have found that there are practically no voids formed in a wholly leather fiber product, and that there are numerous voids formed in a wholly wood fiber product.

It is, therefore, clear that the relative proportion of wood fiber to leather fiber, varying all the way from zero to the desired amount, will be determined by the particular use for which the article is designed. Excellent results have been obtained for wholly leather fiber products where the impregnation is not of paramount importance. However, where impregnation forms a very important feature in the product, a mixture of wood fiber with leather fiber produces the best results. The wood fiber in drying produces the voids hereinbefore mentioned and allows the impregnation to proceed with relative ease and with thoroughness.

I have given the brief summary of numerous experiments which I have conducted not with a view to limiting the invention but with a view of setting forth what I believe to be the principles underlying my discoveries.

In still another mode of carrying out this invention, water need not be used in the beater but instead creosote with a suitable solvent may be employed, or the product may be dipped in creosote to assist in waterproofing the fibers. If the creosote is used in the beater, it has been found that the fibers will not pick up the same amount of water as where water was the liquid employed in the beater. Consequently there is less shrinking when creosote with a suitable solvent or diluent is used in the beater.

It has been found that the strength of the conduit or other article where leather fiber is used, either mixed with wood fiber or used alone, is many times greater than that of a wood fiber tubing.

Another feature of the resulting product is that it picks up less moisture, is considerably tougher, and has an increased life, particularly when used in underground work.

Of paramount importance is the fact that the waste leather is very much cheaper than the wood pulp, whether obtained from paper stock or from other stock. Heretofore this leather scrap has been merely dumped or thrown away and may, therefore, be obtained with a minimum of expense, sometimes, in fact, without cost.

This invention, therefore, supplies a long felt want in providing a very cheap fibrous conduit or article and a method which may be readily followed in the production of such article.

Although this invention has been described in considerable detail, it is to be understood that such description is intended as illustrative rather than limiting, as the invention may be variously embodied and is to be interpreted as claimed.

I claim:

1. The process of making a conduit which comprises disintegrating leather scrap into leather fibers, washing the same, solely with substantially pure water and mixing wood fibers therewith, shaping the mixture of fibers into a conduit, drying the shaped conduit to form voids adjacent the wood fibers, filling the voids with a hot waterproofing material, and subsequently suddenly chilling the impregnated conduit to prevent deformation of the impregnated conduit while it is hot.

2. The process of making a conduit which comprises washing leather scrap solely with substantially pure water to remove the salts from tanning, disintegrating the scrap leather into leather fibers and mixing wood fibers therewith, shaping the mixture of fibers into a conduit, drying the shaped conduit, and impregnating the shaped conduit with a waterproofing material.

3. The process of making a conduit which comprises washing leather scrap thoroughly with warm water, said water being substantially pure and free from any added ingredients, to remove tanning salts and other impurities, disintegrating the leather into fibers, mixing wood fibers therewith, while wet, shaping the resulting wet mixture of fibers into a conduit, drying the shaped conduit and impregnating the dried conduit with a suitable waterproofing material.

4. The process of making a conduit which comprises washing leather scrap thoroughly with warm water, said water being substantially pure and free from any added ingredients to remove tanning salts and other impurities, disintegrating the leather into fibers, mixing wood fibers therewith, while wet, shaping the resulting wet mixture of fibers into a conduit, drying the shaped conduit and impregnating the shaped conduit with a material containing casein and hardening the same with an aldehyde.

CARLTON J. KATZE-MILLER.